

March 25, 1958

**G. R. FINDLAY**

2,828,201

## METHOD FOR PRODUCING TITANIUM AND ZIRCONIUM

Filed Oct. 13, 1950

3 Sheets-Sheet 1



FIG. 1



FIG. 2

INVENTOR.

BY Oliver W. Holmes

Oliver W. Hayes

**ATTORNEY**

March 25, 1958

G. R. FINDLAY

2,828,201

METHOD FOR PRODUCING TITANIUM AND ZIRCONIUM

Filed Oct. 13, 1950

3 Sheets-Sheet 2



FIG. 3

INVENTOR,  
Gordon R. Findlay

BY

Oliver W. Neary

ATTORNEY

March 25, 1958

**G. R. FINDLAY**

2,828,201

## METHOD FOR PRODUCING TITANIUM AND ZIRCONIUM

Filed Oct. 13, 1950

3 Sheets-Sheet 3



FIG. 4

INVENTOR.

BY  
Oliver W. Hayes

ATTORNEY

# United States Patent Office

2,828,201

Patented Mar. 25, 1958

1

2,828,201

## METHOD FOR PRODUCING TITANIUM AND ZIRCONIUM

Gordon R. Findlay, Bedford, Mass., assignor to National Research Corporation, Middlesex County, Mass., a corporation of Massachusetts

Application October 13, 1950, Serial No. 189,917

2 Claims. (Cl. 75—84.4)

This invention relates to the production of metals and more particularly to processes and apparatus for producing metals such as titanium, zirconium, and the like. In my copending application Serial No. 140,339, filed January 24, 1950, now abandoned, there is described a process and apparatus for producing metals wherein a group IVa metal compound, particularly a halide of one of the metals titanium or zirconium, is vaporized and fed into a reaction zone. A reducing metal, preferably sodium or other alkali or alkaline earth metal, is also vaporized and fed into the same reaction zone. The alkaline earth metals include magnesium as well as calcium (see Latimer and Hildebrand, "Reference Book of Inorganic Chemistry," New York, Macmillan Company, 1936 ed., p. 45). For simplicity, the invention will be initially described in connection with the use of alkali metals. The vapors of the group IVa metal halide and the alkali metal are thoroughly intermixed as they enter the reaction zone to form a single stream of the two vapors in which the two vapors burn with intense heat to reduce the metal halide to the group IVa metal and to form a halide of the alkali metal as a by-product. The above process is highly exothermic and requires careful control of the temperatures obtained during the reaction. It also requires careful control of temperatures adjacent the reaction zone so as to permit formation of an ingot of the group IVa metal and to achieve separate condensation of the by-products of the reaction and unreacted starting materials.

It is a principal object of the present invention to provide an improved apparatus and process for practicing the invention described in my above-mentioned copending application.

Another object of the present invention is to provide an improved apparatus of the above type having a high thermal efficiency, ease of control, and simplicity of construction.

Still another object of the invention is to provide novel ingot-casting apparatus and processes which are particularly advantageous for use in forming ingots of metals such as titanium, zirconium, and the like.

Still another object of the present invention is to provide improved temperature control in the production of metals of the above type.

Other objects of the invention will in part be obvious and will in part appear hereinafter.

The invention accordingly comprises the process involving the several steps and the relation and the order of one or more of such steps with respect to each of the others, and the apparatus possessing the construction, combination of elements and arrangement of parts which are exemplified in the following detailed disclosure, and the scope of the application of which will be indicated in the claims.

For a fuller understanding of the nature and objects of the invention, reference should be had to the following detailed description taken in connection with the accompanying drawings wherein:

2

Fig. 1 is a diagrammatic, schematic, sectional view of one preferred form of the invention;

Fig. 2 is a fragmentary view of a portion of the apparatus of Fig. 1 taken along the line 2—2;

Fig. 3 is a flow sheet showing one preferred arrangement of auxiliary equipment and the order of the various steps in the process; and

Fig. 4 is a fragmentary, schematic, sectional view of another embodiment of the invention.

In general this invention relates to the production of metals, and more particularly to the production of metals such as titanium, zirconium, and the like by the reduction of compounds thereof in an air-free atmosphere. For simplicity of illustration the present invention will be described hereinafter in more detail in connection with the reduction of titanium tetrachloride to titanium by sodium vapors, without intending to limit the scope of the invention thereby. For making ingots of titanium, for example, the apparatus of the present invention preferably comprises a reaction chamber and an ingot-forming mold associated with this reaction chamber. Into the reaction chamber there is fed a vapor of a reducible titanium compound, such as titanium tetrachloride. A vaporized metallic reducing agent, such as sodium vapor, is also fed into the reaction chamber, the two feeding means being arranged as a "torch" so that the vapors are intimately mixed as they enter the reaction chamber to cause intense burning of the vapors with the reduction of the titanium tetrachloride to titanium; and with the formation of sodium chloride as a by-product. Associated with the above elements there is provided a means for storing a supply of the metallic reducing agent (i. e., sodium) in molten condition, a means for confining a liquid heat-exchange medium in contact with the walls of the reaction chamber, and a means for controlling the temperature of the walls of the reaction chamber by controlling the rate at which the heat-exchange medium removes heat therefrom. In one preferred embodiment the control of the removal of heat is achieved by a means for controlling the vapor pressure above the liquid heat-exchange medium, thereby controlling the temperature of this liquid heat-exchange medium. In another embodiment of the invention the removal of heat is controlled by controlling the area of contact between the heat-exchange medium and a heat transfer medium in heat-transfer relationship thereto.

In one preferred embodiment of the invention the metallic reducing agent (i. e., the sodium) serves as the heat-exchange medium, and the means for confining the heat-exchange medium in heat-exchange relationship with the walls of the reaction chamber includes at least a portion of the means for storing the supply of the reducing agent. It is also preferred that the vapor pressure controlling means be arranged to maintain the sodium vapor pressure sufficiently high so that the temperature of the sodium in heat-exchange relationship with the walls of the reaction chamber is above the melting point of the sodium chloride formed in the reaction chamber. As a result of this construction the walls of the reaction chamber are maintained at a temperature which is above the melting point of the sodium chloride by-product, and below the temperature at which this sodium chloride has an appreciable vapor pressure. Thus the walls of the reaction chamber serve as a condenser for the sodium chloride by-product.

Referring now more particularly to the drawings, where like numbers refer to like elements in all the figures, the apparatus comprises a reaction vessel 10 defining therewithin a reaction chamber 12. Surrounding the reaction vessel 10 there is preferably positioned a second vessel 14, the space 16 between these two vessels being arranged to hold a liquid heat-exchange medium 18.

Near the bottom of the reaction chamber 12 there is located an ingot-forming mold 20 in which a titanium ingot 21 is formed during the reaction. For achieving intimate mixture of the titanium tetrachloride and sodium vapors there is provided a torch 22 which separately feeds the two vapors into the reaction chamber and directs these two vapors together as they enter the chamber so as to form a flame 23 in which the reduction takes place. This flame 23 serves as the reaction zone and achieves complete reduction of the titanium tetrachloride to metallic titanium. Since the flame 23 is directed towards the ingot mold 20, the resultant titanium is caused to impinge on the surface of an ingot in the mold and to coalesce on this surface, the flame being sufficiently hot to maintain at least the upper surface of the ingot in molten condition.

The reaction chamber 12 includes a vacuum-pumping port 24 connected to a suitable vacuum-pumping system, not shown, which can evacuate the reaction chamber 12 to a low free air pressure on the order of less than .001 mm. Hg abs. Located near the bottom of the reaction chamber, and spaced to one side of the ingot mold, is an outlet pipe 26 for removing liquid sodium chloride 27.

The vapor pressure of the heat-exchange medium 18 is controlled by a pressure relief valve, generally indicated at 28, the setting of this pressure relief valve 28 controlling the temperature of the liquid heat-exchange medium as a function of the vapor pressure in the space 16a thereabove. The liquid heat-exchange medium, as indicated previously, is preferably sodium since sodium has excellent thermal conductivity at high temperatures, and also since it must be vaporized for use in the preferred reaction described above. In the preferred arrangement shown the sodium vapors existing in the space 16a above the surface of the liquid sodium 18 are used as a source of supply for the sodium vapors fed to the torch 22. This torch 22 comprises, in the preferred form shown, a rod 30 preferably formed of a refractory metal, such as molybdenum, having a plurality of holes 32 near the periphery thereof (see Fig. 2). A central hole 34 is also provided in the rod 30, the holes 32 being for the purpose of feeding sodium vapors into the reaction zone, and the hole 34 being for the purpose of feeding titanium tetrachloride vapors into the reaction zone. This torch provides a short flame in which there is through intermixing of the sodium and titanium tetrachloride vapors. This flame 23 is preferably a forced diffusion type of flame which achieves complete reaction, in a highly concentrated zone, between the sodium and titanium tetrachloride vapors. The sodium vapors are fed to the holes 32 by means of a distributing collar 36 in communication with the upper ends thereof, while titanium tetrachloride vapors are fed to the hole 34 by means of a tube 38 connected to the upper end of this hole 34. A pipe 40 leads from the space 16a above the level of the molten sodium, this pipe 40 being connected to the collar 36 and the flow of sodium vapor through this pipe being controlled by a valve 42. This valve 42 is preferably provided with a long stem 44 having an exteriorly positioned operating handle 46 and a water-cooled seal 48.

The pressure relief valve 28 for controlling the vapor pressure of the sodium in the chamber 16 comprises a valve 52, the degree of opening of which is controlled by a pressure responsive device, such as a spring 54. A pipe 56 is included for permitting escape, to a suitable receptacle, of excess sodium vapors generated in space 16a by the exothermic reaction which occurs within the reaction chamber 12.

The mold 20 in which the titanium ingot 21 is formed comprises a curved flange portion 60 surrounding a central cylindrical portion 62, these two portions being preferably integral and formed of a refractory metal, such as molybdenum. At the bottom of the central cylindrical section 62 there is included a reducing die 64 which reduces the diameter of the titanium ingot 21 as it

is withdrawn by a pair of rolls 656. This reducing die 64 thus serves as a vacuum seal to prevent passage of air into the reaction zone between the boundaries of the forming ingot and the mold surface. Surrounding the mold is a liquid sodium guide 66 which serves to cause flow of liquid sodium into heat-exchange relationship with the exterior surfaces of mold portions 60 and 62, this sodium being introduced through a pipe 68 and, in one preferred form of the invention, the entering liquid sodium being at a lower temperature than the remainder of the sodium 18 in the space 16 so as to remove heat from the mold walls at a high rate.

A sight tube 70 is positioned near the top of the reaction chamber, this sight tube extending through the inner and outer vessels 10 and 14 respectively, and through a layer of insulation 72 which preferably surrounds the whole apparatus. At the top of the sight tube there is provided a sight glass 74 adjacent to which is positioned a water-cooling coil 76. Argon or other inert gas is preferably introduced through a pipe 78 so as to cause a flow of argon gas down the sight tube 70 to remove any vapors which might otherwise diffuse up the tube 70 and condense either as a smoke within tube 70 or as a coating on the inner surface of the sight glass 74. The sight glass 74 is preferably also provided with a wiper (not shown) for removing from the inner surface of the sight glass any condensed material which reaches the sight glass despite the argon flow.

The preferred operation of the device of Fig. 1, and 30 the arrangement of the auxiliary equipment, is illustrated best in the flow diagram of Fig. 3 wherein like numbers refer to like elements in the other figures. In this Fig. 3 there is provided a storage chamber 80 for holding the 35 reducible metal compound A (e. g. titanium tetrachloride). A supply tank for holding the molten metallic reducing agent B (e. g. sodium) is indicated at 82. A 40 pump or valve 84 is included for feeding the titanium tetrachloride from the supply 80 to a vaporizer 86 therefor, while a pump or valve 88 is included for transferring molten sodium from supply 82 to the space 16 surrounding the reaction vessel 10. For electrolyzing the 45 sodium chloride reaction product the pipe 26 leads to an electrolysis chamber 90, the sodium formed in this chamber 90 being piped to supply 82 through a filter 91 for 50 removing impurities such as oxides. The chlorine generated in chamber 90 is piped to a reaction vessel 92 in which the titanium tetrachloride is formed by reaction with titanium dioxide and carbon. This manufacture of titanium tetrachloride is well described in chapter 17 of 55 "Titanium, Its Occurrence, Chemistry and Technology" by Barksdale, published (1949) by the Ronald Press Co., New York. The resultant crude titanium tetrachloride is then piped to a crude storage tank 93 at which point a purifying agent such as oleic acid may be added. From 60 the crude storage tank the crude titanium tetrachloride goes to a stripper 94 where some impurities, such as silicon tetrachloride, are removed. It then passes through a fractionation column 95, and the thus purified titanium tetrachloride is then pumped to storage chamber 80. 65 For initially heating the sodium in the space 16 to a desired high temperature on the order of 1000° C. there is provided a heater 96 which heats the sodium to 1000° C., the vapors of the sodium condensing at the top of the space 16 and the condensed sodium being recirculated 70 through the heater until the sodium in space 16 has been brought up to the desired temperature. If desired, separate condensers 97 and 98, for unreacted sodium and unreacted titanium tetrachloride, respectively, may be provided in the vacuum pumping line 24 leading to a vacuum pumping system schematically indicated at 99.

In the operation of the device shown in Figs. 1, 2, and 3, the supply chambers 80 and 82 are filled with titanium tetrachloride and sodium, respectively, some of the sodium being fed to space 16 so as to fill this space to the 75 level indicated. Heater 96 is energized to heat the sodium

in space 16 to the desired temperature, preferably about 1000° C. During the heat-up time the reaction chamber 12 is preferably being evacuated by means of vacuum pump 99 to a free air pressure on the order of less than about 1 micron Hg abs. In lieu of evacuating chamber 12 it may be purged of air by sweeping with argon introduced through pipe 78 at a pressure slightly in excess of atmospheric pressure.

When the reaction chamber 12 has been brought to its desired temperature of about 1000° C. the feed of argon through pipe 78 and down the sight tube 70 is commenced. The valve 42 is opened to allow sodium vapors to enter the distributing collar 36 and to pass down the outer holes 32 in the torch 22. At the same time the titanium tetrachloride is fed into the pipe 38 by pumping titanium tetrachloride from the supply tank 80 to the vaporizer 86. The thus vaporized titanium tetrachloride enters the central hole 34 in the torch 22 and mixes intimately with the sodium as the two vapors issue from the end of the torch. The feed of the sodium and the titanium tetrachloride vapors is preferably accomplished with a stoichiometric relationship therebetween. If desired an excess of sodium may be fed to the reaction zone, this excess being helpful in preventing formation of lower chlorides resulting from incomplete reduction of the titanium tetrachloride. During the travel of the titanium tetrachloride vapor down pipe 38 and through the hole 34 in the torch, this vapor is preferably superheated by the heat of the reaction chamber to a temperature on the order of about 1000° C. The two hot vapors issuing from the end of the torch ignite with a highly exothermic reaction to give an intensely hot flame 23 in which the sodium reduces the titanium tetrachloride to metallic titanium with sodium chloride as a by-product. The flame temperature is preferably about 2000° C. so that the titanium formed therein is subjected to a temperature above its melting point. This flame is directed towards the top of the ingot 21 in the mold 20 and maintains the upper surface of this titanium ingot in molten condition. The metallic titanium formed by the reduction reaction is driven by the flame, and the initial velocity of the reactants, towards the surface of the ingot where it coalesces on the surface of this ingot. Since the temperature of the flame 23 is extremely high the by-product sodium chloride 27 remains in the vapor phase and is completely separated from the metallic titanium formed in the flame. The sodium chloride 27 is condensed on the walls of the reaction chamber, runs down these walls and is withdrawn from the reaction chamber 12 by means of pipe 26. This sodium chloride 27 passes to the electrolysis chamber 90 where it is electrolyzed, by usual techniques, to sodium and chlorine. The resultant sodium is recirculated to the sodium supply 82 while the chlorine is passed to the reaction chamber for forming titanium tetrachloride by reaction with carbon and titanium dioxide. This titanium tetrachloride is then purified and fed to the titanium tetrachloride supply 80. Any unreacted sodium and titanium tetrachloride are separately condensed in condensers 97 and 98 and fed back to their respective supplies.

During the reaction the total pressure in the system is maintained at about atmospheric pressure by the argon which travels down sight glass tube 70, this argon being removed at a constant rate by the pump 99. The vapor pressure of the sodium in space 16 is maintained essentially constant during the process by the operation of the pressure relief valve 28. The sodium vapors which pass through pressure relief valve 28 are condensed in condenser 97 and then fed back to the sodium supply 82. The heat of condensation of the sodium may conveniently be utilized for vaporizing the titanium tetrachloride and maintaining the sodium supply molten by use of a suitable heat-exchange device (not shown).

As the titanium, formed in the flame 23, coalesces on

the upper surface of the ingot 21 in the mold 20, the size of the ingot increases. Consequently, the ingot is withdrawn by rolls 65 as the titanium is added to the ingot, the level of the top of the ingot being preferably kept constant during this withdrawal. The control of the ingot withdrawal may be achieved by the use of thermocouples (not shown) which measure the temperature in the mold wall 62 and thus indicate the level of titanium therein.

Referring now to Fig. 4 there is shown another embodiment of the invention which is of particular value for those installations where it is undesirable to control high-temperature sodium vapor pressures by use of a pressure relief valve. In this embodiment of the invention, where like numbers refer to like elements in the preceding figures, there are three separate bodies of heat-exchange liquid concentrically arranged around the reaction chamber. The second body of heat-exchange liquid serves as a variable-area heat-transfer medium between the first and third bodies of heat-exchange liquid. The effective area 20 of the heat-transfer medium between the first and third heat-exchange liquids is preferably controlled as a direct function of the vapor pressure above the first heat-exchange liquid (i. e. that body of heat-exchange liquid closest to the reaction chamber). In a preferred form 25 of this embodiment the first and second bodies of heat-exchange liquid are two portions of the sodium supply.

The main body of the sodium is in contact with the walls of the reaction chamber and the other portion is between the main body and the third body of heat-exchange liquid, this second portion of sodium serving as the variable-area heat-exchange medium. As the vapor pressure (and temperature) of the main body of sodium rises it forces some of the sodium into the second body thereof to increase the area of the second body of sodium 30 between the main body and the third body of heat-exchange liquid, thus increasing the rate of heat removal from the main body of liquid sodium.

In Fig. 4 there is provided a third vessel 100 outside of vessel 14, vessel 100 forming a third chamber 102 in which a relatively small body of sodium 18a is confined, there being small passages 104 between chambers 102 and 16. Outside of vessel 100 is a fourth vessel 106 defining a fourth chamber 108 with the vessel 100 for holding a third heat-exchange liquid 110. The space 112 above liquid sodium 18a is filled with a predetermined inert gas pressure to maintain a pressure difference above the two bodies of sodium 18 and 18a. Space 114 above the heat-exchange liquid 110 is filled with vapors of this liquid 110. For controlling the level of sodium 18 in chamber 16 there is a level-responsive device, such as a resistance element 116, connected to a measuring means 118. The measuring means 118 is preferably arranged to control a valve 120 in the sodium feed line 68. The vapor pressure in space 114 is controlled by a pressure relief valve 122 to allow escape of the vapors of liquid 110 from space 114 to prevent heat-exchange liquid 110 from reaching a temperature above its decomposition point. The condensed heat-exchange liquid is fed back into chamber 108 by means of a pipe 124.

The operation of the Fig. 4 arrangement is essentially the same as the operation of the apparatus described in Figs. 1, 2, and 3, with the difference, however, that the control of the temperature of the wall of the reaction chamber is achieved in a somewhat modified manner. In Fig. 4 the change in the vapor pressure of the sodium 18 adjacent the reaction chamber is used to control the removal of heat by changing the rate of heat transfer from this sodium 18. The level of the sodium 18 is maintained substantially constant by the resistance element 116, the measuring system 118, and the valve 120. In a preferred arrangement the valve 120 is normally open sufficiently to permit the entrance of an amount of sodium equal to that being used by the process. Any 70 changes in the level of sodium in chamber 16 then cause

a correcting change in the amount of opening of valve 120.

In the Fig. 4 embodiment of the invention the heat-exchange liquid 110 is preferably "Dowtherm" (a eutectic mixture of phenyl ether and diphenyl) and the heat imparted thereto is utilized to heat the titanium tetrachloride, maintain the sodium in liquid condition, and to heat steam for power purposes where there is considerable excess heat available. In both the Fig. 1 and Fig. 4 embodiments of the invention, the various parts of the apparatus are preferably constructed of 310 stainless steel except the torch 22 and mold 60, 62, which are preferably made of molybdenum.

While the invention has been specifically described in connection with the use of the preferred titanium tetrachloride as the reducible product-metal compound and the preferred sodium as the metallic reducing agent, numerous other materials may be employed. The essential attributes for the metallic reducing agent (B in Fig. 3), which enable it to achieve a satisfactory reduction of a reducible product-metal halide, are set forth below:

(1) The heat of reaction of the metallic reducing agent with the reducible product-metal halide must be great enough, at a temperature corresponding to the melting point of the product metal, to supply at least enough heat for:

(a) the total heat capacity of the reactant materials and the by-products of the reaction between the preheat temperature and the melting point of the product metal;

(b) the heat of vaporization of the by-product halide of the metallic reducing agent;

(c) the heat of fusion of the product-metal;

(d) the heat loss in the "cold mold" 20 or its equivalent; and

(e) the radiation heat loss from the reaction flame.

(2) The free energy change of the reaction ( $\Delta F$ ), at a temperature corresponding to the melting point of the product-metal, must be favorable or a satisfactory yield must be possible by regulation of the pressure at which the reaction is carried out.

(3) The vapor pressure of the halide of the metallic reducing agent, which is a by-product of the reaction, shall be high in comparison with the vapor pressure of the product-metal at the melting point of the product-metal so as to achieve vaporization of this halide of the metallic reducing agent.

(4) The vapor pressure of the metallic reducing agent should be high because of the necessity for:

(a) vaporizing the metallic reducing agent for the reaction; and

(b) preventing the metallic reducing agent from remaining in the product-metal, particularly if there is any appreciable solubility of the two metals.

(5) The chosen metallic reducing agent should have no solubility, or very little solubility, in the product-metal at the melting point of the product-metal and, in addition, the metallic reducing agent should not react with the product-metal to form intermetallic compounds.

(6) It is not essential, but it is considered important from an economic standpoint, that the metallic reducing agent

(a) have a low melting point;

(b) have a small ratio of atomic weight to valence;

(c) be easy to prepare from its halide by means such as electrolysis;

(d) be capable of being prepared in, or purified to, a high state of purity free from nitrides and oxides in particular;

(e) be noncorrosive or nonreactive with available materials of construction at the temperatures required;

(f) be relatively abundant so that the capital investment in metallic reducing agent required for circulation in the system be low;

(g) have good thermal conductivity; and

(h) have a low heat of vaporization.

In preferred forms of the invention the reducible product-metal compound (A in Fig. 3) is a product-metal halide and preferably meets the following requirements:

(1) The product-metal halide is preferably volatile and preferably has a boiling point less than about 800° C. The product-metal halide does not decompose into lower halides at its volatilization temperature.

(2) The product-metal halide must be capable of being purified to a high degree to remove product-metal oxide or oxyhalide salts. The product-metal should have a vapor pressure or boiling point substantially different from any oxide or oxyhalide salt that the product-metal might form so that purification of the product-metal halide can be effected by distillation.

(3) The product-metal should have a vapor pressure which is low at its melting point and is low with respect to the pressure in the reaction zone to minimize loss of the product-metal by evaporation.

(4) The product-metal halide should have a satisfactory high heat of reaction with the chosen reducing agent.

When materials other than the preferred titanium tetrachloride and sodium are used, the temperature of the walls of the reaction chamber is adjusted so that it is above the melting point of the by-product compound formed during the reducing reaction and below that temperature at which the vapor pressure of the by-product compound is an appreciable portion of the total pressure in the reaction chamber. In order to achieve the above operating conditions it is only necessary to control the rate of heat removal by controlling the vapor pressure above the heat-exchange medium surrounding the reaction chamber in the Fig. 1 form of the invention, or by adjusting the heat-transfer area of the intermediate heat-exchange liquid in the Fig. 4 embodiment.

While the invention has been described primarily in connection with the manufacture of pure metals, it is equally adaptable to the manufacture of alloys. In this latter case a mixture of two reducible metal compounds may be fed into the reaction zone through the pipe 38 so that the two metallic compounds may be simultaneously reduced to form the desired binary alloy. Equally, tertiary and quaternary alloys may be formed, if desired, by the above process. Accordingly, the word "metal" used in the appended claims is intended to include alloys as well as the pure metal.

Since certain changes may be made in the above process and apparatus without departing from the scope of the invention herein involved, it is intended that all matter contained in the above description, or shown in the accompanying drawings, shall be interpreted as illustrative and not in a limiting sense.

What is claimed is:

1. In a process for producing a group IV metal from the class consisting of titanium and zirconium by reduction of a group IV metal tetrahalide with a metallic reducing agent from the group consisting of the alkali metals and the alkaline earth metals, the improvement which comprises mixing vapors of the tetrahalide and vapors of the reducing agent in a reaction zone in a reaction chamber so that the vapors react with intense heat to form a highly heated reaction flame which is at a temperature above the melting point of the group IV metal and above the vaporization temperature of the by-product halide, directing said reaction flame against the surface of the group IV metal body to maintain said surface molten by transfer of heat from the flame to the surface and to collect on the molten group IV metal surface liquid group IV metal carried in the flame, simultaneously removing heat from the group IV metal body to solidify liquid group IV metal at the solid-liquid interface, separately withdrawing the product group IV metal and the by-product halide from the reaction zone, confining a first liquid heat-exchange medium in contact with, and outside of, the walls of a reaction chamber, maintaining a second liquid heat-exchange medium in

heat-transfer relationship between said first heat-exchange medium and a third heat-exchange medium, and controlling the degree of heat transfer through said second heat-exchange medium as a direct function of the vapor pressure of said first heat-exchange medium.

2. In a process for producing a group IV metal from the class consisting of titanium and zirconium by reduction of a group IV metal tetrahalide with a metallic reducing agent from the group consisting of the alkali metals and the alkaline earth metals, the improvement which comprises mixing vapors of the tetrahalide and vapors of the reducing agent in a reaction zone in a reaction chamber so that the vapors react with intense heat to form a highly heated reaction flame which is at a temperature above the melting point of the group IV metal and above the vaporization temperature of the by-product halide, directing said reaction flame against the surface of the group IV metal body to maintain said surface molten by transfer of heat from the flame to the surface and to collect on the molten group IV metal surface liquid group IV metal carried in the flame, simultaneously removing heat from the group IV metal body to solidify liquid group IV metal at the solid-liquid interface, separately withdrawing the product group IV metal and the by-product halide from the reaction zone, and

5

10

20

25

controlling the removal of heat from said reaction chamber by regulating the pressure of the vapor of a heat-exchange liquid confined in heat-exchange relationship with the outside of the reaction chamber.

References Cited in the file of this patent

UNITED STATES PATENTS

|           |                   |                |
|-----------|-------------------|----------------|
| 1,305,726 | Leonard           | June 3, 1919   |
| 1,306,568 | Weintraub         | June 10, 1919  |
| 1,499,852 | Cerini            | July 1, 1924   |
| 1,519,582 | Harris            | Dec. 16, 1924  |
| 1,670,965 | Heron             | May 22, 1928   |
| 1,698,624 | Dale              | Jan. 8, 1929   |
| 1,747,070 | Grafflin          | Feb. 11, 1930  |
| 1,748,518 | Midgley           | Feb. 25, 1930  |
| 1,840,588 | Knox              | Jan. 12, 1932  |
| 1,894,982 | Eppensteiner      | Jan. 24, 1933  |
| 1,929,520 | Rudorff           | Oct. 10, 1933  |
| 2,365,194 | Hodson et al.     | Dec. 19, 1944  |
| 2,482,127 | Schlechten et al. | Sept. 20, 1949 |
| 2,564,337 | Maddex            | Aug. 14, 1951  |

FOREIGN PATENTS

253,161 Great Britain June 7, 1926